

Specimens.)

F. W. FARNHAM.

MATCH

No. 335,065.

Patented Jan. 26, 1886

Fig. 1.



Fig. 2.



Witnesses:

F. W. Farnham,  
J. J. McElhenny.

Inventor:

Frederick W. Farnham  
by S. W. Seely  
Atty.

# UNITED STATES PATENT OFFICE.

FREDERICK W. FARNHAM, OF WHITE MILLS, PENNSYLVANIA, ASSIGNOR TO  
EUNICE A. FARNHAM, OF SAME PLACE.

## MATCH.

SPECIFICATION forming part of Letters Patent No. 335,065, dated January 26, 1886.

Application filed July 7, 1884. Serial No. 137,003. (Specimens.)

To all whom it may concern:

Be it known that I, FREDERICK W. FARNHAM, a citizen of the United States, residing at White Mills, in the county of Wayne and State of Pennsylvania, have invented certain new and useful Improvements in Matches, of which the following is a specification, reference being had therein to the accompanying drawings.

10 My invention relates to an improvement in friction-matches; and the object of my invention is to produce a match which will be practically safe in use, and yet will be capable of ignition upon any convenient frictional surface.

15 The ordinary parlor-match in use consists of a thick heavy splint tipped with a large round head of inflammable material. When struck sharply on a frictional surface, it is well known to all that particles of the head are liable to be thrown off in any direction, and as these particles are always ignited they are dangerous to the person or dress of the person who lights them. Such matches are often struck upon gas-brackets upon a level with the eyes, which are thus put in danger from these flying particles. Again, such matches, if stepped on carelessly, will ignite directly with a large flame, dangerous to 20 the dresses of ladies, and always a source of risk.

25 My invention consists in a match having a two-part head or compound tip composed of different compositions, the larger part attached to the splint being composed of a safety composition which will ignite only from contact with flame, or by friction upon a specially-prepared surface, while the extreme tip is composed of a small portion of 30 igniting composition which will light when struck upon any frictional surface.

35 I prefer to use my device in connection with the invention shown and described in my Patent No. 303,564, of August 12, 1884, where-  
40 in the invention is a series or strip of partly-separated match-splints tipped with an igniting composition and partly coated with a frictional surface; but my present invention is applicable as well for single matches, and I do

not limit myself to any particular form of match or any particular ignitable compositions.

The invention is illustrated in the drawings, in which Figure 1 is a view of a single match made according to my invention. Fig. 55 2 shows a strip of matches of the kind shown in my application referred to, but tipped according to my present invention.

A represents a match-splint the upper end of which is preferably tapered, as at a. This match is tipped with any suitable safety composition, b—such as a mixture of twenty-four parts of chlorate of potash, two parts of ultramarine-blue, and sixteen parts of black sulphate of antimony. This composition will 60 ignite only upon its proper frictional surface, or in the presence of actual flame, and cannot be ignited by being stepped on, or by careless handling of any kind. At tip the extreme point of this head b with a very small portion of an 65 igniting composition, composed, for instance, of five parts of ordinary phosphorus, eight parts of saltpeter, fifteen parts of yellow ocher or brick-dust, with sufficient glue, gum, or starch to give the compound adhesiveness. 70 This tip is of a different color from the main head, and can be ignited in the usual way; but it is not large enough to throw off any particles, and produces just sufficient flame to 75 ignite the safety composition. It will not ignite when the match is stepped on, because the safety composition will crumble off, being 80 so much larger than the ignitable tip.

In Fig. 2 I have shown my compound head as applied to a strip of partly-separated 85 matches provided with a frictional surface, c.

Having described my invention, I claim—

A match having a head composed of two separate compounds, one a safety composition and the other or tip an ordinary frictionally- 90 ignitable composition.

In testimony whereof I affix my signature in presence of two witnesses.

FREDERICK W. FARNHAM.

Witnesses:

F. G. FARNHAM,  
F. C. FARNHAM.